

## UNITED STATES PATENT OFFICE.

RALPH E. BATEMAN, OF DAYTON, OHIO.

## ART OF APPLYING DECORATIVE COATINGS.

No Drawing.

Application filed February 4, 1924. Serial No. 690,652.

*To all whom it may concern:*

Be it known that I, RALPH E. BATEMAN, a citizen of the United States of America, residing at Dayton, county of Montgomery, 5 and State of Ohio, have invented certain new and useful Improvements in the Art of Applying Decorative Coatings, of which the following is a full, clear, and exact description.

10 This invention relates to the art of applying paint coatings to surfaces, especially decorative coatings to metal surfaces.

An object of this invention is to provide a simple and inexpensive method of applying 15 a paint coating to a surface to produce a desired rough finish such as a pebble, imitation leather, egg shell, or other similar finish.

Another object is to provide a simple 20 method of producing such a finish in two or more colors.

Another object is to provide a method of reducing the tendency of the spattered rough coating to flow out smooth while drying, thus greatly increasing the "coarseness" 25 of the rough coating which may be obtained by this invention.

Further objects will be apparent from the 30 following detailed description of the invention. It is not thought that the invention can be aptly illustrated by drawings.

The material used for forming the rough, irregular, or what will herein be termed the "spatter" coating may be any rapid drying 35

paint mixture of such a consistency that it will pass through the atomizing device used in relatively large globules and form a spatter effect upon the surface being coated. A kind of paint well known under the trade 40 name of "Duco" is particularly suitable for use in the method of this invention as it does not have to be mixed with any additional material to produce good results. Of course, however, the degree of coarseness of

45 the "spatter" coating may be varied by thinning out the paint mixture with any suitable rapid drier. Another paint mixture which has been used with success in the method of this invention is an approximately half and half mixture of paint color ground in japan and a quick drier known under the trade name of "Fibroseal." Also a half and half mixture of color ground in

japan and Viscolac gives good results. These two materials are well mixed to form 55 a paste which is only fluid enough to go through the atomizing device used and form a spatter effect upon the surface to be coated. For forming a very coarse spatter coating a thicker paste is used and 60 the atomizing device is adjusted accordingly to permit the passage of larger globules of paste therethrough. The atomizing device used in this invention may be any suitable and well 65 known form of air brush commonly used for applying smooth coats of paint or varnish by spraying out a fine spray of the paint or varnish upon the surface to be coated therewith until the entire surface is covered with 70 a smooth regular coat. When used in the method of this invention, however, the air brush should be adjusted to permit a freer passage for the paint mixture therethrough in order that relatively large globules of 75 thick paint mixture may pass through and be deposited upon the surface to be coated. Of course these globules are deposited upon the surface in a very irregular and haphazard pattern. The coarseness 80 of the globules may be adjusted to give a pebble, leather, egg shell, or mat finish or any degree thereof. It has been found preferable in most cases to apply a priming coating to the surface and permit it to dry before the application of the above-described 85 spatter coating.

The surface upon which the spatter coating is applied should preferably be in a substantially horizontal position in order to 90 reduce the tendency of the deposited globules to flow by gravity over the surface while drying and thus become distorted. The quick drying property of the mixture causes the globules to become so viscous 95 immediately after being deposited that they will not melt away as is the case with ordinary paints and varnishes but will dry in the form of globules substantially as they are first deposited. When applying the 100 coating to small articles such as umbrella handles, brushes, hand mirrors, lamps, small containers, or any small article where it is desired to finish the entire article without waiting for one surface of the article to dry 105 before applying to another surface thereof,

this invention contemplates revolving the article about a substantially horizontal axis at a speed which will prevent the globules from flowing down and becoming distorted by gravity. In the case of substantially cylindrical articles, the articles may be revolved upon their own axis at quite a rapid rate since in this case the globules will not be impelled by centrifugal force to move laterally over the cylindrical surface.

When it is desired to give a mottled two color coating to a surface, the first spatter coating of the desired base color is applied in the manner above described and permitted to dry. The second coating of the desired different color may then be applied on top of the spatter coating by an ordinary brush or rubbed on with a piece of cloth so that the second color is well applied to the low surfaces or valleys in the spatter coating. The second color is easily removed from the high surfaces of the spatter coating while it is still wet by rubbing with a cloth, or by any other easily devised method, thus exposing the first color at all the high areas. It is thus obvious that a two color irregularly mottled coating may be applied to an originally smooth surface by means of paint without having to roughen the surface itself in any way.

While the process as herein disclosed, constitutes a preferred form of the invention, it is to be understood that other forms might be adopted, all coming within the scope of the claims which follow.

What is claimed is as follows:

1. The method of coating metal surfaces comprising: first priming the surface to be coated with a priming coating, then applying a rapid drying paint mixture to said surface by means of an air brush, said mixture being of such consistency that it flows from the air brush in globules and forms a pebble effect upon said surface, and then drying said last coating before it has sufficient time to become smooth.

2. The method of coating metal surfaces comprising: first priming the surface to be coated with a priming coating, then applying a rapid drying paint mixture to said surface by blowing relatively large globules of said mixture onto said surface with an atomizing device, and then permitting said globules to dry quickly, whereby said surface retains a permanently roughened irregular coating of paint.

3. The method of coating surfaces comprising: applying a rapid drying paint mixture to said surface by means of an air brush, said mixture being of such consistency that it flows from the air brush in globules and forms a pebble effect upon said surface, and then drying said coating before it has sufficient time to become smooth.

4. The method of coating surfaces com-

prising: applying a rapid drying paint mixture to said surface by blowing relatively large globules of said mixture onto said surface with an atomizing device, and then permitting said globules to dry quickly, whereby said surface retains a permanently roughened irregular coating of paint.

5. The method of applying paint upon a surface to give an imitation leather effect comprising: applying a rapid drying paint mixture to said surface by blowing globules of said mixture thereon with an atomizing device, and then permitting said mixture to dry quickly, whereby said surface retains a permanently irregular coating of paint.

6. The method of applying paint upon a surface to give an imitation leather effect comprising: first applying a base coating to said surface, then applying a rapid drying paint mixture to said surface by blowing globules of said mixture thereon with an atomizing device, and then permitting said mixture to dry quickly, whereby said surface retains a permanently irregular coating of paint.

7. The method of giving surfaces a mottled two-color coating comprising: first applying a smooth priming coating, then applying a rapid drying thick paint mixture by blowing globules of said mixture onto said surface with an atomizing device, permitting said last coating to dry quickly to give a roughened surface, and then applying a coating of a different color and rubbing said last coating down while wet to remove said last coating from the high surfaces of the rough coating.

8. The method of giving surfaces a mottled two-color coating comprising: applying a rapid drying thick paint mixture by blowing globules of said mixture onto said surface with an atomizing device, permitting said coating to dry quickly to give a roughened surface, and then applying a coating of a different color and rubbing said last coating down while wet to remove said last coating from the high surfaces of the rough coating.

9. The method of applying paint to surfaces including: applying a rapid drying thick paint mixture by blowing globules of said mixture onto a surface, permitting said applied paint to dry quickly before the globules have time to flow out and form a smooth coating, then applying a coating of different colored paint over the rough globules thus formed and removing the second coating from the high spots on the rough globules.

10. The method of coating a surface including: applying a rapid drying thick paint mixture by blowing globules of said paint onto a surface and changing the angular position of the surface relative to the

horizontal while said globules are drying to face about a non-vertical axis while said globules are drying to reduce the tendency of the globules to flow out and become smooth while drying.

11. The method of coating a surface including: applying a rapid drying thick paint mixture by blowing globules of said paint onto a surface and revolving said surface about a non-vertical axis while said globules are drying to reduce the tendency of the globules to flow out and become smooth while in a fluid state.

In testimony whereof I hereto affix my signature.

RALPH E. BATEMAN.